



US010953468B2

(12) **United States Patent**  
**Thakare**

(10) **Patent No.:** **US 10,953,468 B2**  
(45) **Date of Patent:** **Mar. 23, 2021**

(54) **POLYCRYSTALLINE DIAMOND  
COMPOSITE COMPACT ELEMENTS AND  
METHODS OF MAKING AND USING SAME**

(71) Applicant: **Element Six (UK) Limited**,  
Oxfordshire (GB)

(72) Inventor: **Mandar Rajiv Thakare**, Oxfordshire  
(GB)

(73) Assignee: **Element Six (UK) Limited**,  
Oxfordshire (GB)

(\*) Notice: Subject to any disclaimer, the term of this  
patent is extended or adjusted under 35  
U.S.C. 154(b) by 0 days.

(21) Appl. No.: **16/631,793**

(22) PCT Filed: **Jul. 17, 2018**

(86) PCT No.: **PCT/EP2018/069357**  
§ 371 (c)(1),  
(2) Date: **Jan. 16, 2020**

(87) PCT Pub. No.: **WO2019/016190**

PCT Pub. Date: **Jan. 24, 2019**

(65) **Prior Publication Data**

US 2020/0180033 A1 Jun. 11, 2020

(30) **Foreign Application Priority Data**

Jul. 17, 2017 (GB) ..... 1711417

(51) **Int. Cl.**  
**B22F 7/06** (2006.01)  
**B22F 3/12** (2006.01)  
(Continued)

(52) **U.S. Cl.**  
CPC ..... **B22F 7/062** (2013.01); **B22F 3/12**  
(2013.01); **B22F 7/08** (2013.01); **C22C 26/00**  
(2013.01);  
(Continued)

(58) **Field of Classification Search**

None

See application file for complete search history.

(56) **References Cited**

U.S. PATENT DOCUMENTS

5,662,183 A 9/1997 Fang  
6,013,117 A 1/2000 Ederyd  
(Continued)

FOREIGN PATENT DOCUMENTS

WO 200196050 A2 12/2001  
WO 2006032982 A1 3/2006  
(Continued)

OTHER PUBLICATIONS

International Search Report and Written Opinion issued for PCT/EP2018/069357, dated Sep. 17, 2018 (12 pages).

(Continued)

*Primary Examiner* — Bryan D. Ripa

*Assistant Examiner* — Ross J Christie

(74) *Attorney, Agent, or Firm* — Armstrong Teasdale LLP

(57) **ABSTRACT**

A polycrystalline diamond (PCD) composite compact element has a body of polycrystalline diamond material and a cemented carbide substrate bonded to the body of polycrystalline material along an interface. The cemented carbide substrate has tungsten carbide particles bonded together by a binder material, the binder material including an alloy of Co, Ni and Cr. The tungsten carbide particles form at least 70 weight percent and at most 95 weight percent of the substrate and the binder material has between about 60 to 90 wt. % Ni, between about 10 to 40 wt. % Co, and about 0.25 to 1.0 wt %  $\text{Cr}_3\text{C}_2$ .

**11 Claims, 2 Drawing Sheets**



- (51) **Int. Cl.**
- |                    |           |                                         |            |
|--------------------|-----------|-----------------------------------------|------------|
| <i>B22F 7/08</i>   | (2006.01) | 2015/0111065 A1* 4/2015 Konyashin ..... | C22C 29/16 |
| <i>C22C 26/00</i>  | (2006.01) |                                         | 428/682    |
| <i>C22C 29/06</i>  | (2006.01) | 2016/0325404 A1* 11/2016 Long .....     | B24D 3/06  |
| <i>C22C 29/08</i>  | (2006.01) | 2016/0326809 A1* 11/2016 Long .....     | C22C 11/00 |
| <i>E21B 10/573</i> | (2006.01) |                                         |            |
- (52) **U.S. Cl.**
- |           |                                                                                                                                                                                        |                         |  |
|-----------|----------------------------------------------------------------------------------------------------------------------------------------------------------------------------------------|-------------------------|--|
| CPC ..... | <i>C22C 29/067</i> (2013.01); <i>C22C 29/08</i> (2013.01); <i>E21B 10/5735</i> (2013.01); <i>B22F 2998/10</i> (2013.01); <i>B22F 2999/00</i> (2013.01); <i>C22C 2026/006</i> (2013.01) | WO 2013087773 A1 6/2013 |  |
|           |                                                                                                                                                                                        | WO 2017114677 A1 7/2017 |  |

(56) **References Cited**

## U.S. PATENT DOCUMENTS

- |                   |                                      |              |
|-------------------|--------------------------------------|--------------|
| 8,727,045 B1 *    | 5/2014 Mukhopadhyay .... E21B 10/573 | 175/434      |
| 9,039,798 B2 *    | 5/2015 Lai Sang .....                | B22F 3/14    |
|                   |                                      | 51/309       |
| 2010/0303565 A1   | 12/2010 Xiao et al.                  |              |
| 2013/0048389 A1 * | 2/2013 Bao .....                     | B24D 18/0009 |
|                   |                                      | 175/428      |
| 2014/0165476 A1 * | 6/2014 Can .....                     | E21B 10/54   |
|                   |                                      | 51/309       |

- |                                         |            |
|-----------------------------------------|------------|
| 2015/0111065 A1* 4/2015 Konyashin ..... | C22C 29/16 |
|                                         | 428/682    |
| 2016/0325404 A1* 11/2016 Long .....     | B24D 3/06  |
| 2016/0326809 A1* 11/2016 Long .....     | C22C 11/00 |

## FOREIGN PATENT DOCUMENTS

- |    |               |        |
|----|---------------|--------|
| WO | 2013087773 A1 | 6/2013 |
| WO | 2017114677 A1 | 7/2017 |

## OTHER PUBLICATIONS

- Combined Search and Examination Report issued for GB1711417. 4, dated Jan. 16, 2018 (9 pages).
- Combined Search and Examination Report issued for GB1811657. 4, dated Sep. 25, 2018 (8 pages).
- International Standard, "Microbeam Analysis—Electron Backscatter Diffraction—Measurement of Average Grain Size," International Organization for Standardization, ISO 13067:2011(E) (26 pages).
- Roebuck, "Magnetic Moment (Saturation) Measurements on Hardmetals," International Journal of Refractory Metals and Hard Materials, 14(5-6): 419-424 (1996).

\* cited by examiner



FIG. 1

TWL in mg



FIG. 2



FIG. 3

## 1

**POLYCRYSTALLINE DIAMOND  
COMPOSITE COMPACT ELEMENTS AND  
METHODS OF MAKING AND USING SAME**

**CROSS-REFERENCE TO RELATED  
APPLICATIONS**

This application is a § 371 national stage of International Application No. PCT/EP2018/069357, filed Jul. 17, 2018, which claims priority to Great Britain Application No. 1711417.4, filed Jul. 17, 2017.

**FIELD**

This disclosure relates to polycrystalline diamond (PCD) composite compact elements, tools incorporating the same, and methods for making and using the same.

**BACKGROUND**

Polycrystalline diamond (PCD) is a super-hard, also known as superabrasive, material comprising a mass of inter-grown diamond grains and interstices between the diamond grains. PCD may be made by subjecting an aggregated mass of diamond grains to an ultra-high pressure and temperature. A material wholly or partly filling the interstices may be referred to as filler material. PCD may be formed in the presence of a sintering aid such as cobalt, which is capable of promoting the inter-growth of diamond grains. The sintering aid may be referred to as a solvent/catalyst material for diamond, owing to its function of dissolving diamond to some extent and catalysing its re-precipitation. A solvent/catalyst for diamond is understood to be a material that is capable of promoting the growth of diamond or the direct diamond-to-diamond inter-growth between diamond grains at a pressure and temperature condition at which diamond is thermodynamically stable. Consequently the interstices within the sintered PCD product may be wholly or partially filled with residual solvent/catalyst material. PCD may be formed on a cobalt-cemented tungsten carbide substrate, which may provide a source of cobalt solvent/catalyst for the PCD.

PCD may be used in a wide variety of tools for cutting, machining, drilling or degrading hard or abrasive materials such as rock, metal, ceramics, composites and wood-containing materials. For example, PCD elements may be used as cutting elements on drill bits used for boring into the earth in the oil and gas drilling industry. Such cutting elements for use in oil and gas drilling applications are typically formed of a layer of PCD bonded to a cemented tungsten carbide-cobalt substrate and, in many of these applications, the temperature of the PCD material may become elevated as it engages a rock formation, workpiece or body with high energy. Unfortunately, mechanical properties of PCD such as hardness and strength tend to deteriorate at high temperatures, largely as a result of residual solvent/catalyst material dispersed within it. Another major problem experienced with such cutters is the relatively low erosion resistance of the carbide substrate of the cutter. This may result in the carbide substrate being eroded very quickly during the drilling process due to mud forming from the coolants used in the drilling process and penetration of abrasive particles from the drilled rock into the carbide substrate. A worn and eroded carbide substrate cannot support the PCD layer attached thereto, with the result that the whole cutter may fail.

## 2

Furthermore, current market conditions are dictating that drill bits are pushed further and harder with the ability to re-use a cutter at least once (preferably twice) being required. Erosion to the cutter substrate results in an irregular fit between cutter and the pocket in the drill bit into which the cutter is brazed, and this irregular fit may affect the braze bond and therefore cutter retention. Severe erosion may therefore prevent the re-use (spinning) of cutters which has the downstream effect of deteriorating the rental economics for the bit manufacturer.

The practical use of cemented carbide grades with substantially lower cobalt content as substrates for PCD inserts is limited by the fact that some of the Co is required to migrate from the substrate into the PCD layer during the sintering process in order to catalyse the formation of the PCD and a reduced amount of cobalt in the substrate has conventionally therefore been considered disadvantageous as it may adversely affect the sintering of the PCD, thereby weakening the inter-bonding of the diamond grains. For this reason, it has been conventionally more difficult to make PCD on substrate materials comprising lower Co contents, even though this may be desirable.

There is therefore a need for cemented carbide substrates for attachment to a body of PCD material having improved erosion and/or corrosion resistance that do not have an adverse effect on the sintering quality of the PCD.

**SUMMARY**

Viewed from a first aspect there is provided a polycrystalline diamond (PCD) composite compact element comprising:

a body of polycrystalline diamond material; and  
a cemented carbide substrate bonded to the body of polycrystalline material along an interface;  
the cemented carbide substrate comprising tungsten carbide particles bonded together by a binder material, the binder material comprising an alloy of Co, Ni and Cr; the tungsten carbide particles forming at least 70 weight percent and at most 95 weight percent of the substrate; wherein the binder material comprises between about 60 to 90 wt. % Ni, between about 10 to 40 wt. % Co, and about 0.25 to 1.0 wt %  $\text{Cr}_3\text{C}_2$ .

Viewed from a second aspect there is provided a method of making the above defined polycrystalline diamond (PCD) composite compact element, the method comprising:

providing tungsten carbide powder;  
milling the tungsten carbide powder with a binder to form a blended powder;  
compacting the blended powder to form a green body;  
sintering the green body to produce the cemented carbide body;  
bonding the cemented carbide body to a body of polycrystalline diamond material by:  
forming an assembly comprising a plurality of diamond grains, the cemented carbide body and a binder material for the polycrystalline diamond;  
subjecting the assembly to a sufficiently high temperature for the binder material to be in the liquid state and to a first pressure at which diamond is thermodynamically stable;  
reducing the pressure to a second pressure at which the diamond is thermodynamically stable, the temperature being maintained sufficiently high to maintain the binder material in the liquid state;  
reducing the temperature to solidify the binder material; and

reducing the pressure and the temperature to an ambient condition to form a body of polycrystalline diamond material bonded to the cemented carbide body.

#### BRIEF DESCRIPTION OF THE DRAWINGS

Various versions will now be described by way of example and with reference to the accompanying drawings in which:

FIG. 1 is an EBSD image of tungsten carbide grains dispersed in a sintered cemented carbide body according to an example;

FIG. 2 is a plot of potential against current density in a static corrosion test of an example and a conventional cutter; and

FIG. 3 is a chart showing the results of a mass loss erosion-corrosion test for an example cutter and a conventional cutter.

#### DETAILED DESCRIPTION

As used herein, a “catalyst material for diamond”, also referred to as “solvent/catalyst for diamond”, is a material that is capable of promoting the nucleation, growth or inter-bonding of diamond grains at a pressure and temperature at which diamond is thermodynamically stable. Catalyst materials for diamond may be metallic, such as cobalt, iron, nickel, manganese and alloys of these, or non-metallic.

As used herein, “polycrystalline diamond” (PCD) material comprises a mass of diamond grains, a substantial portion of which are directly inter-bonded with each other and in which the content of diamond is at least about 80 volume percent of the material. In one embodiment of PCD material, interstices between the diamond gains may be at least partly filled with a binder material comprising a catalyst for diamond. As used herein, “interstices” or “interstitial regions” are regions between the diamond grains of PCD material. In embodiments of PCD material, interstices or interstitial regions may be substantially or partially filled with a material other than diamond, or they may be substantially empty. As used herein, a “filler” material is a material that wholly or partially fills pores, interstices or interstitial regions within a structure, such as a polycrystalline structure. Thermally stable embodiments of PCD material may comprise at least a region from which catalyst material has been removed from the interstices, leaving interstitial voids between the diamond grains. As used herein, a “thermally stable PCD” structure is a PCD structure at least a part of which exhibits no substantial structural degradation or deterioration of hardness or abrasion resistance after exposure to a temperature above about 400 degrees centigrade.

As used herein, the grain sizes are expressed in terms of Equivalent Circle Diameter (ECD) according to the ISO FDIS 13067 standard. The ECD is obtained by measuring of the area A of each grain exposed at the polished surface and calculating the diameter of a circle that would have the same area A, according to the equation  $ECD=(4A/\pi)^{1/2}$  (See section 3.3.2 of ISO FDIS 13067 “Microbeam analysis—Electron Backscatter Diffraction—Measurement of average grain size.”, International Standards Organisation Geneva, Switzerland, 2011).

Example PCD composite compact elements may comprise a PCD structure bonded along an interface to a cemented carbide substrate comprising particles of a metal carbide and a metallic binder material.

An example of a PCD composite compact element may be made by a method including providing a cemented carbide substrate, contacting an aggregated, substantially unbonded mass of diamond particles against a surface of the substrate 5 to form an pre-sinter assembly, encapsulating the pre-sinter assembly in a capsule for an ultra-high pressure furnace and subjecting the pre-sinter assembly to a pressure of at least about 5.5 GPa and a temperature of at least about 1,250 degrees centigrade, and sintering the diamond particles to 10 form a PCD composite compact element comprising a PCD structure integrally formed on and joined to the cemented carbide substrate. In some versions, the pre-sinter assembly may be subjected to a pressure of at least about 6 GPa, at least about 6.5 GPa, at least about 7 GPa or even at least 15 about 7.5 GPa.

The hardness of cemented tungsten carbide substrate may be enhanced by subjecting the substrate to an ultra-high pressure and high temperature, particularly at a pressure and temperature at which diamond is thermodynamically stable.

20 The magnitude of the enhancement of the hardness may depend on the pressure and temperature conditions. In particular, the hardness enhancement may increase the higher the pressure. Whilst not wishing to be bound by a particular theory, this is considered to be related to the Co drift from the substrate into the PCD during press sintering, as the extent of the hardness increase is directly dependent 25 on the decrease of Co content in the substrate.

In some examples such as where the PCD structure is 30 integrally formed onto the substrate during sintering at an ultra-high pressure, solvent/catalyst material may be included or introduced into the aggregated mass of diamond grains from a source of the material other than the cemented carbide substrate. The solvent/catalyst material may comprise cobalt that infiltrates from the substrate in to the 35 aggregated mass of diamond grains just prior to and during the sintering step at an ultra-high pressure.

In some examples, solvent/catalyst for diamond may be 40 introduced into the aggregated mass of diamond grains by various methods, including blending solvent/catalyst material in powder form with the diamond grains, depositing solvent/catalyst material onto surfaces of the diamond grains, or infiltrating solvent/catalyst material into the aggregated mass from a source of the material other than the substrate, either prior to the sintering step or as part of the 45 sintering step. Methods of depositing solvent/catalyst for diamond, such as cobalt, onto surfaces of diamond grains are well known in the art, and include chemical vapour deposition (CVD), physical vapour deposition (PVD), sputter coating, electrochemical methods, electroless coating methods and atomic layer deposition (ALD). It will be appreciated that the advantages and disadvantages of each depend 50 on the nature of the sintering aid material and coating structure to be deposited, and on characteristics of the grain.

In one example of a method, cobalt may be deposited onto 55 surfaces of the diamond grains by first depositing a precursor material and then converting the precursor material to a material that comprises elemental metallic cobalt. For example, in the first step cobalt carbonate may be deposited on the diamond grain surfaces using the following reaction:



The deposition of the carbonate or other precursor for cobalt or other solvent/catalyst for diamond may be achieved by means of a method described in PCT patent publication number WO/2006/032982. The cobalt carbonate may then be converted into cobalt and water, for example, by means of pyrolysis reactions such as the following:



In another example, cobalt powder or precursor to cobalt, such as cobalt carbonate, may be blended with the diamond grains. Where a precursor to a solvent/catalyst such as cobalt is used, it may be necessary to heat treat the material in order to effect a reaction to produce the solvent/catalyst material in elemental form before sintering the aggregated mass.

It has now been unexpectedly appreciated that if the binder phase of cemented carbides contains nickel and chromium in a pre-determined proportion, the erosion resistance of cemented carbides may be dramatically improved without adversely affecting the quality of the PCD to which the carbide forms a substrate in the sintering process. Also, the Vickers hardness, transverse rupture strength, indentation fracture toughness and wear-resistance of the cemented carbides containing the pre-determined proportions of nickel and chromium may be noticeably increased.

In some examples, the cemented carbide substrate may be formed of tungsten carbide particles bonded together by the binder material, the binder material comprising an alloy of Co, Ni and Cr. The tungsten carbide particles may form at least 70 weight percent and at most 95 weight percent of the substrate. The binder material may comprise between about 60 to 90 wt. % Ni, between about 10 to 40 wt. % Co, and around 0.25 to 1.0 wt %  $\text{Cr}_3\text{C}_2$ . In one example, the binder material may comprise around 59.5 wt % Ni, around 40 wt % Co and around 0.5 wt %  $\text{Cr}_3\text{C}_2$ . In some examples, the binder additionally comprises between about 2 to 20 wt. % tungsten and between about 0.1 to 2 wt. % carbon. In some examples, the binder material may comprise between about 60 to 70 wt. % Ni, between about 30 to 40 wt. % Co, and, in some examples additionally around 0.25 to 0.5 wt %  $\text{Cr}_3\text{C}_2$ .

In terms of the substrate, in some examples, the cobalt content may comprise between around 3 to 10 wt %, such as around 5 wt %, the nickel may comprise between around 5 to 10 wt % such as around 7.5 wt % and the  $\text{Cr}_3\text{C}_2$  may comprise between around 0.2 to 1 wt % such as 0.5 wt %, the remainder comprising tungsten and carbon.

The magnetic properties of the cemented carbide material may be related to important structural and compositional characteristics. The most common technique for measuring the carbon content in cemented carbides is indirectly, by measuring the concentration of tungsten dissolved in the binder to which it is indirectly proportional: the higher the content of carbon dissolved in the binder the lower the concentration of tungsten dissolved in the binder. The tungsten content within the binder may be determined from a measurement of the magnetic moment,  $a$ , or magnetic saturation,  $M_s = 4\pi\sigma$ , these values having an inverse relationship with the tungsten content (Roebuck (1996), "Magnetic moment (saturation) measurements on cemented carbide materials", *Int. J. Refractory Met.*, Vol. 14, pp. 419-424). The following formula may be used to relate magnetic saturation,  $M_s$ , to the concentrations of W and C in the binder:

$$M_s \propto [C]/[W] \times \text{wt. \% Co} \times 201.9 \text{ in units of } \mu\text{T} \cdot \text{m}^3/\text{kg}$$

The binder cobalt content within a cemented carbide material may be measured by various methods well known in the art, including indirect methods such as such as the magnetic properties of the cemented carbide material or more directly by means of energy-dispersive X-ray spectroscopy (EDX), or a method based on chemical leaching of Co.

The mean grain size of carbide grains, such as WC grains, may be determined by examination of micrographs obtained using a scanning electron microscope (SEM) or light microscopy images of metallurgically prepared cross-sections of a cemented carbide material body, applying the mean linear intercept technique, for example. Alternatively, the mean size of the WC grains may be estimated indirectly by measuring the magnetic coercivity of the cemented carbide material, which indicates the mean free path of Co intermediate the grains, from which the WC grain size may be calculated using a simple formula well known in the art. This formula quantifies the inverse relationship between magnetic coercivity of a Co-cemented WC cemented carbide material and the Co mean free path, and consequently the mean WC grain size. Magnetic coercivity has an inverse relationship with MFP.

In some examples, the cemented carbide substrate may have a mean magnetic coercivity of at least about 100 Oe and at most about 145 Oe.

As used herein, the "mean free path" (MFP) of a composite material such as cemented carbide is a measure of the mean distance between the aggregate carbide grains cemented within the binder material. The mean free path characteristic of a cemented carbide material may be measured using a micrograph of a polished section of the material. For example, the micrograph may have a magnification of about 1500 $\times$ . The MFP may be determined by measuring the distance between each intersection of a line and a grain boundary on a uniform grid. The matrix line segments,  $L_m$ , are summed and the grain line segments,  $L_g$ , are summed. The mean matrix segment length using both axes is the "mean free path". Mixtures of multiple distributions of tungsten carbide particle sizes may result in a wide distribution of MFP values for the same matrix content.

The concentration of W in the Co binder depends on the C content. For example, the W concentration at low C contents is significantly higher. The W concentration and the C content within the Co binder of a Co-cemented WC (WC-Co) material may be determined from the value of the magnetic saturation. The magnetic saturation  $4\pi\sigma$  or magnetic moment  $\sigma$  of a hard metal, of which cemented tungsten carbide is an example, is defined as the magnetic moment or magnetic saturation per unit weight. The magnetic moment,  $\sigma$ , of pure Co is 16.1 micro-Tesla times cubic metre per kilogram ( $\mu\text{T} \cdot \text{m}^3/\text{kg}$ ), and the induction of saturation, also referred to as the magnetic saturation,  $4\pi\sigma$ , of pure Co is 201.9  $\mu\text{T} \cdot \text{m}^3/\text{kg}$ .

A desired MFP characteristic may be accomplished several ways known in the art. For example, a lower MFP value may be achieved by using a lower metal binder content. A practical lower limit of about 3 weight percent cobalt applies for cemented carbide and conventional liquid phase sintering. In an embodiment where the cemented carbide substrate is subjected to an ultra-high pressure, for example a pressure greater than about 5 GPa and a high temperature (greater than about 1,400 °C, for example), lower contents of metal binder, such as cobalt, may be achieved. For example, where the cobalt content is about 3 weight percent and the mean size of the WC grains is about 0.5 micron, the MFP would be about 0.1 micron, and where the mean size of the WC grains is about 2 microns, the MFP would be about 0.35 microns, and where the mean size of the WC grains is about 3 microns, the MFP would be about 0.7 microns. These mean grain sizes correspond to a single powder class obtained by natural comminution processes that generate a log normal distribution of particles. Higher matrix (binder) contents would result in higher MFP values.

Changing grain size by mixing different powder classes and altering the distributions may achieve a whole spectrum of MFP values depending on the particulars of powder processing and mixing. The exact values would have to be determined empirically.

In some examples, the body of polycrystalline diamond material comprises Co, Ni and Cr.

The binder material may include at least about 0.1 weight percent to at most about 5 weight percent one or more of V, Ta, Ti, Mo, Zr, Nb and Hf in solid solution.

A polycrystalline diamond (PCD) composite compact element according to some examples may have a specific weight loss in an erosion test in a recirculating rig generating an impinging jet of liquid-solid slurry below  $2 \times 10^{-3}$  g/cm<sup>3</sup> at the following testing conditions: a temperature of 50° C., an impingement angle of 45°, a slurry velocity of 20 m/s, a pH of 8.02, a duration of 3 hours, and a slurry composition in 1 cubic meter water of: 40 kg Bentonite; 2 kg Na<sub>2</sub>CO<sub>3</sub>; 3 kg carboxymethyl cellulose, 5 litres.

Some examples of a cemented carbide body may be formed by providing tungsten carbide powder having a mean equivalent circle diameter (ECD) size in the range from about 0.2 microns to about 0.6 microns, the ECD size distribution having the further characteristic that fewer than 45 percent of the carbide particles have a mean size of less than 0.3 microns; 30 to 40 percent of the carbide particles have a mean size of at least 0.3 microns and at most 0.5 microns; 18 to 25 percent of the carbide particles have a mean size of greater than 0.5 microns and at most 1 micron; fewer than 3 percent of the carbide particles have a mean size of greater than 1 micron. The tungsten carbide powder is milled with binder material comprising Co, Ni and Cr or chromium carbides, the equivalent total carbon comprised in the blended powder being, for example, about 6 percent with respect to the tungsten carbide. The blended powder is then compacted to form a green body and the green body is sintered to produce the cemented carbide body. In some example, the substrate further comprises free carbon.

The sintering the green body may take place at a temperature of, for example, at least 1,400 degrees centigrade and at most 1,440 degrees centigrade for a period of at least 65 minutes and at most 85 minutes.

The size distribution of the tungsten carbide powder may, in some examples, have the characteristic of a mean ECD of 0.4 microns and a standard deviation of 0.1 microns.

Versions are described in more detail below with reference to the example below which is not intended to be limiting.

#### Example

A batch of carbide substrates for PCD was produced by a conventional powder metallurgy route. First, a 5 kg powder mixture was produced. A WC powder was milled with 9.75 wt. % Co powder with mean grain size of nearly 1.5 µm, 2.95 wt. % Ni powder with mean grain size of roughly 2.5 µm and 0.3 wt. % Cr<sub>3</sub>C<sub>2</sub> powder with mean grain size 1.6 µm in a ball mill with 30 kg carbide balls and 100 g paraffin wax. Once the powder had been dried, it was granulated and compacted to form substrates for PCD in the form of green bodies.

The green bodies were sintered by means of a Sinterhip™ furnace at 1,420 degrees centigrade for about 75 min, 45 min of which was carried out in vacuum and 30 min of which was carried out in a HIP apparatus in an Ar at a pressure of about 40 bars. Afterwards a layer of polycrystalline diamond

was obtained on the carbide substrates by use of conventional procedures using high-pressure and high-temperatures to produce PCD cutters.

After this, metallurgical cross-sections of the cutters were made and the composition of a layer of the carbide substrate adjacent to the PCD layer was examined by mean of energy-dispersive X-ray microanalysis (EDX). Also the PCD layer was cut off and the magnetic properties of the carbide substrates were examined.

The size distribution of the WC grains in the starting WC powder was measured as follows. The WC powder was blended with 50 weight percent Cu powder and the resulting blend was compacted and sintered at 1,100 degrees centigrade in a vacuum for 30 min. As it is known that WC does not substantially dissolve in Cu or react with Cu, the original size distribution of the WC is preserved within the Cu matrix. The sintered Cu-based body was sectioned and prepared for microscopic metallurgical analysis, and the size distribution of the WC grains embedded in the Cu matrix was measured.

Electron Backscatter Diffraction (EBSD) images were obtained by means of a high-resolution scanning electron microscope (HRSEM). The grain sizes were obtained and are expressed in terms of Equivalent Circle Diameter (ECD) according to the ISO FDIS 13067 standard. The ECD is obtained by measuring of the area A of each grain exposed at the polished surface and calculating the diameter of a circle that would have the same area A, according to the equation ECD=(4A/π)<sup>1/2</sup> (See section 3.3.2 of ISO FDIS 13067 "Microbeam analysis—Electron Backscatter Diffraction—Measurement of average grain size.", International Standards Organisation Geneva, Switzerland, 2011). The mean grain sizes of WC grains of the original WC powder was equal to 0.4 µm and in the sintered cemented carbide was equal to 0.6 µm. The grain size distributions of the grains in the original WC powder and sintered cemented carbide are shown in Table 1.

TABLE 1

| sample                    | Grain size distribution of WC in the sintered cemented carbide and original powder. |            |            |            |         |
|---------------------------|-------------------------------------------------------------------------------------|------------|------------|------------|---------|
|                           | <0.3 µm                                                                             | 0.3-0.5 µm | 0.5-1.0 µm | 1.0-1.5 µm | >1.5 µm |
| Sintered cemented carbide | 13.5%                                                                               | 23.6%      | 53.7%      | 8.7%       | 0.5%    |
| Original WC               | 39.8%                                                                               | 35.4%      | 22.9%      | 1.7%       | 0.2%    |

The magnetic coercivity of the carbide substrates was found to be equal to roughly 139 Oe and their magnetic moment to be equal to 10.9 Gcm<sup>3</sup>/g. The Vickers hardness of the substrates was equal to HV10=1210.

The cemented carbide substrates were examined in an erosion test in a recirculating erosion-corrosion rig generating impinging jet of liquid-solid slurry and in situ electrochemical monitoring apparatus that allowed high velocity liquid impingement on test samples. The following testing conditions were applied: temperature of 50° C., impingement angle of 90°, slurry flow velocity 15 m/s, pH of between 3, duration of 3 hrs, slurry composition in 1 cubic meter water: sand 40 g and 3.5% NaCl in solution. The results of this test are shown in FIG. 2.

Also, conventional cemented carbide substrates with 13 wt. % Co not containing chromium and nickel were examined in the same test on erosion resistance. Table 2 shows the

WC grain size distribution of the conventional grade indicating that there are much more grains with grain sizes of 1.0 to 1.5  $\mu\text{m}$  and significantly more abnormally large WC grains with a grain size of more than 1.5  $\mu\text{m}$ . The wide range of WC grain size distribution with a large number of large and abnormally large WC grains in the conventional cemented carbide is expected to result in a decreased combination of hardness, fracture toughness, and wear and erosion resistance.

TABLE 2

| Grain size distribution of WC in the conventional cemented carbide |                    |                       |                       |                       |                    |
|--------------------------------------------------------------------|--------------------|-----------------------|-----------------------|-----------------------|--------------------|
| sample                                                             | <0.3 $\mu\text{m}$ | 0.3-0.5 $\mu\text{m}$ | 0.5-1.0 $\mu\text{m}$ | 1.0-1.5 $\mu\text{m}$ | >1.5 $\mu\text{m}$ |
| Sintered cemented carbide                                          | 9.4%               | 15.7%                 | 49.3%                 | 21.1%                 | 4.5%               |

The magnetic coercivity of the carbide substrates was found to be equal to roughly 109 Oe and their magnetic moment to be equal to  $20.5 \text{ Gcm}^3/\text{g}$ , which is equal to 98.0% of the theoretical value for nominally pure Co. The Vickers hardness of the substrates was equal to HV10=1210.

As shown in FIG. 2, the specific weight loss of the conventional cemented carbide (denoted by reference numeral 1) in the erosion-resistance test described above was significantly more than the mass loss of the carbide made according to the example (denoted by reference numeral 2), therefore the erosion resistance of the cemented carbide according to an example was higher than that of the conventional one by roughly a factor of 2.

Furthermore, it was determined that the PCD of the compact made according to the example was well sintered with good diamond to diamond interbonding.

The cemented carbide substrates of the example and above described conventional substrate were also examined in a Static Corrosion Test which is a linear polarisation resistance method developed by Stern and Geary (1957) which measured corrosion rate under steady state conditions. Linear polarisation techniques assume that in activation controlled systems, the exponential anodic and cathodic polarisation curves are approximate to a straight line close to the free corrosion potential. A small external DC potential signal of  $\pm 10$  to 20 mV is applied to the system, and the current flowing in the external circuit is measured. For similar current densities, a higher corrosion potential would suggest an improved resistance to corrosion. The results are shown in FIG. 3 with the results for the carbide formed according to the example being denoted by reference numeral 10 and those for the conventional cemented carbide by reference numeral 20.

Whilst not wishing to be bound by a particular theory, it is believed that some examples may significantly improve the erosion resistance of carbide by employing a cemented carbide in combination with a Co-based binder alloyed with a high percentage of chromium and nickel. This is found to

lead to improved performance of a PCD cutter comprising a body of PCD material bonded to the carbide substrate, without adversely affecting the sintering of the PCD body.

The invention claimed is:

1. A polycrystalline diamond (PCD) composite compact element comprising:
  - a body of polycrystalline diamond material; and
  - a cemented carbide substrate bonded to the body of polycrystalline material along an interface;
  - the cemented carbide substrate comprising tungsten carbide particles bonded together by a binder material, the binder material comprising an alloy of Co, Ni and Cr; the tungsten carbide particles forming at least 70 weight percent and at most 95 weight percent of the substrate; wherein the binder material comprises between about 60 to 90 wt. % Ni, between about 10 to 40 wt. % Co, and about 0.25 to 1.0 wt %  $\text{Cr}_3\text{C}_2$ ; and
  - wherein the binder material additionally comprises between about 2 to 20 wt. % tungsten and between about 0.1 to 2 wt. % carbon.
2. A polycrystalline diamond (PCD) composite compact element according to claim 1, wherein the binder material comprises between about 60 to 70 wt. % Ni, between about 0.25 to 1 wt. %  $\text{Cr}_3\text{C}_2$ , and between around 30 to 40 wt % Co.
3. A polycrystalline diamond (PCD) composite compact element according to claim 1 wherein the layer of substrate further comprises free carbon.
4. A polycrystalline diamond (PCD) composite compact element according to claim 1, wherein the body of polycrystalline diamond material comprises Co, Ni and Cr.
5. A polycrystalline diamond (PCD) composite compact element as claimed in claim 1, wherein the binder material includes at least about 0.1 weight percent to at most about 5 weight percent one or more of V, Ta, Ti, Mo, Zr, Nb and Hf in solid solution.
6. A polycrystalline diamond (PCD) composite compact element as claimed in claim 1, wherein the Co of the binder material comprises between around 3 to 10 wt % of the substrate, the Ni of the binder material comprises between around 5 to 10 wt % of the substrate, and the  $\text{Cr}_3\text{C}_2$  of the binder material comprises between around 0.2 to 0.5 wt % of the substrate.
7. A tool comprising a PCD composite compact element according to claim 1, the tool being for cutting, milling, grinding, drilling, earth boring, rock drilling or other abrasive applications.
8. A tool according to claim 7, wherein the tool comprises a drill bit for earth boring or rock drilling.
9. A tool according to claim 7, wherein the tool comprises a rotary fixed-cutter bit for use in oil and gas drilling.
10. A tool according to claim 7, wherein the tool is a rolling cone drill bit, a hole opening tool, an expandable tool, a reamer or other earth boring tools.
11. A drill bit or a cutter or a component therefor comprising the PCD composite compact element according to claim 1.

\* \* \* \* \*